# EUROPEAN PATENT SPECIFICATION

(11) **EP 0 315 725 B1**
(45) Date of publication and mention of the grant of the patent: **13.05.1992**
(21) Application number: 87830398.1
(22) Date of filing: 11.11.1987
(51) Int. Cl.: D06P 3/14, D06P 1/44, D06M 15/00, D06M 13/00

(54) **Method of dyeing woollen fabrics and items of clothing to produce a shot effect**
Färbeverfahren zur Herstellung von changierender Wollstückware
Procédé de coloration de tissus de laine en pieces pour produire une effet changeant

(43) Date of publication of application: 17.05.1989
(73) Proprietor: SILLI, Alessandro, I-50047 PRATO (Firenze) (IT)
(72) Inventor: SILLI, Alessandro, I-50047 PRATO (Firenze) (IT)
(74) Representative: Pederzini, Paolo

(56) References cited:
- AU-B- 444 066
- GB-A- 211 178
- GB-A- 1 124 344
- JOURNAL OF THE SOCIETY OF DYERS AND COLOURISTS, vol. 93, no. 1, January 1977, pages 12-14, Bradford, GB; P.R. BRADY et al.: "The coloration of wool fabrics with pigments"
- TEXTILE PROGRESS, vol. 4, no. 3, 1972, pages 1-89, Manchester, GB; T. SHAW et al.: "The finishing of wool fabrics"
- JOURNAL OF THE SOCIETY OF DYERS AND COLOURISTS, vol. 89, no. 9, September 1973, pages 333-334, Bradford, GB; G.B. GUISE et al.: "Attempts to produce bright whites on wool by application of pigments"

## Description

The invention concerns a method of dyeing shot woollen fabrics and items of clothing, hereinafter called "the products" for short.

The aim of the present invention is to dye the products in such a way as to produce a shot effect which causes the colour of the products themselves to change when viewed from different angles, in accordance with she varying angle of incidence of the light rays.

The method as claimed below achieves this shot effect by dyeing or colouring the fibres of the product fabric, and not the surface filaments of the fibres themselves. At the end of the dyeing process, the sad filaments retain a natural white sheen and form a downy "nap" which hides the true colour of the woven fibres from view and creates different colour effects depending on the angle from which the products are viewed.

Basically, the method consists in dyeing the products in two stages, first in water in a rotary dyeing vat, without fixing the dye to the fabric, followed by rinsing, and then placing the products in a second bath, again with the dyeing vat in motion, in order to fix the dye with an elastomer activated by a catalyst.

The two basic stages of the method are described in more detail below.

First of all, the products are dry cleaned before undergoing the dyeing treatment, and are placed in a rotary dyeing vat in a bath of purified water in the ratio of 40 litres of water to every 1 kg of product. Size, is added to the bath in the proportion of 10% of the weight of the products to be dyed. The dyeing vat is made to rotate and heated to a temperature of 50°C, allowing it to continue rotating for 30 minutes.

Colorant is then added to the bath in variable proportions, depending on the desired colour intensity to be achieved, diluted with a dispersing agent. The dyeing vat is further heated to a temperature of 95°C and allowed to continue rotating for 60 minutes.

At the end of the first stage envisaged by the present method, the dyebath is cooled to 50°C, the vat drained of the dyeing solution and the products rinsed.

The second stage consists in fixing the dye to the products treated in the previous stage.

To do this, the products are placed in a bath of clean water, again with the dyeing vat in motion, to which an elastomer is added. The proportion of elastomer for the fixing bath is 10% of the amount of water used.

During rinsing and during the bath with the elastomeric bonding agent, the colorant that had settled on the surface filaments of the product fibres comes off the said filaments and settles on the body of the said fibres.

Subsequently, a catalyst is added to the bath in order to activate the binding action of the elastomer and, consequently, to fix the dye to the product fibres. During experiments on the method, the ideal proportion of catalyst to obtain this pH was found to be 1% of the amount of water for the fixing bath. The products are allowed to remain in this bath, with the dyeing vat in motion, for 30 minutes.

At the end of the second stage, the dyeing vat is drained, the products rinsed (if there are any impurities to be removed), together with a softening agent, if necessary, and finally dried, at 140°C and transferred to subsequent processes.

## Claims

1. A method of dyeing shot woolen fabrics and items of clothing which may be implemented using a rotary dyeing tank, colorants and bonding agents to fix the colorants to the fibres of the products to be dyed, the said method being characterized by the following stages:
a) dyeing the products which have been first drycleaned in a bath of water in a ratio of 40 litres of water to every 1 kg of product, adding to the bath in successive steps firstly a size in a ratio of 10% of the weight of the products, heating the vat to a temperature of 50°C and making it rotate for 30 minutes, and adding secondly a colorant diluted in a dispersing agent and then heating the vat to 95°C and making it rotate for a further 60 minutes;
b) cooling the vat to 50°C, with the vat rotating, and rinsing the treated products; placing the products, treated according to step a), in a bath of clean water, adding to the bath an elastomer in the proportion of 10% of the amount of water used, subsequently activating the elastomer by adding a catalyst to the bath in the proportion of 1% of the amount of water used, and allowing the dyeing vat to rotate for a further 30 minutes; rinsing the products, which are then centrifuged and thoroughly dried at 140° C.

## Revendications

1. Procédé de coloration de tissus de laine en pièces pour produire un effet changeant, à exécuter moyennant l'utilisation d'une cuve de teinturerie à rotation, ainsi que de pigments et de produits de liaison pour la fixation des pigments aux fibres des produits à teindre, ledit procédé étant caractérisé par les étapes suivantes:
a) teinture des produits, qui ont été précédemment nettoyés à sec, dans un bain d'eau suivant un rapport de 40 litres d'eau par chaque kilo de produit, en y ajoutant par étapes en succession d'abord un apprêt dans la proportion de 10% par rapport au poids des produits, chauffant la cuve à une température de 50°C et causant sa rotation pendant 30 minutes, et ensuite un pigment dilué dans un produit dispersant, chauffant la cuve jusqu'à 95°C et causant encore sa rotation pendant 60 minutes;
b) refroidissement de la cuve à 50°C, pendant que la cuve est en rotation, et rinçage des produits traités; placement des produits traités suivant l'étape a) dans un bain d'eau claire en ajoutant au bain un élastomère dans la proportion de 10% de la quantité d'eau utilisée, en activant ensuite l'élastomère moyennant l'adjonction dans le bain d'un catalyseur dans une proportion de 1% de la quantité d'eau utilisée et faisant tourner la cuve de teinturerie pendant 30 minutes encore; rinçage des produits qui seront ensuite centrifugés et complètement séchés à 140°C.

## Patentansprüche

1. Färbeverfahren zur Herstellung von changierender Wollstückware und Bekleidungsteilen, das unter Verwendung eines rotierenden Färbebehälters sowie von Farbstoffen und Fixiermitteln zum Fixieren der Farbstoffe an den Fasern der zu färbenden Produkte durchgeführt wird, dadurch gekennzeichnet, dass das genannte Verfahren folgende Phasen umfasst:
a) Färben der zuvor trockengereinigten Produkte in einem Wasserbad im Verhältnis von 40 l Wasser auf jedes Kilo Produkt, wobei zu aufeinanderfolgenden Zeiten zunächst ein Leim im Verhältnis von 10% des Produktgewichtes beigegeben, der Behälter auf eine Temperatur von 50°C aufgeheizt und für 30 Minuten in Umdrehung versetzt wird, und zweitens ein mit einem Dispergierprodukt verdünnter Farbstoff hinzugefügt und dann der Behälter auf 95°C aufgeheizt und für 60 Minuten in Umdrehung versetzt wird;
b) Abkühlen des Behälters auf 50°C - bei drehendem Behälter - und Spülen der behandelten Produkte; Eintauchen der nach Phase a) behandelten Produkte in ein Bad aus klarem Wasser und Zugabe zu dem Bad eines Elastomers im Verhältnis von 10% der verwendeten Gesamtmenge an Wasser, sowie anschliessendes Aktivieren des Elastomers durch Zugabe eines Beschleunigers im Verhältnis von 1% der verwendeten Gesamtmenge an Wasser, und zwar unter Drehen des Färbebehälters für weitere 30 Minuten; Spülen der Produkte, welche dann bei 140°C durch und durch getrocknet werden.
